

## UNITED STATES PATENT OFFICE

2,598,729

## PREPARATION OF DRYING OILS

Howard M. Teeter, Peoria, Ill., assignor to the  
United States of America as represented by the  
Secretary of Agriculture

No Drawing. Application August 7, 1950,  
Serial No. 178,162

11 Claims. (Cl. 260—405.5)

(Granted under the act of March 3, 1883, as  
amended April 30, 1928; 370 O. G. 757)

1

The invention herein described may be manufactured and used by or for the Government of the United States of America for governmental purposes throughout the world without the payment to me of any royalty thereon.

This invention relates in general to the conversion of non-drying oils to drying oils or more broadly, to the treatment of esters of aliphatic acids containing at least 8 carbon atoms in the acyl radical to increase the olefinic unsaturation thereof, particularly the conjugated unsaturation. In the case of semi-drying oils or non-drying oils the drying properties of said oils are materially enhanced. The invention relates, in particular, to an improved method for removing the halogen substituents of a halogenated glyceride oil whereby the olefinic unsaturation of said oil is increased.

Among the known methods for treating glyceride oils to improve the drying properties thereof, it is conventional procedure to first halogenate and then remove the halogen to effect unsaturation. In the past, various methods have been suggested for both the halogenation and halogen-removing steps. The present invention relates to the second, halogen-removing step, and generally involves treating a halogen-containing glyceride oil with aqueous solutions of weakly basic reacting salts. I have discovered that my novel method of halogen removal produces an oil with markedly improved drying properties. The invention is remarkably simple and easy to carry out, at the same time being relatively low in cost.

Prior methods of halogen removing, particularly dehydrohalogenation of long chain fatty acid compounds, such as esters, and, more particularly, esters of polyhydric alcohols, such as glycerol, have involved thermal treatment by which hydrohalic acids are evolved; or treatment with relatively strong bases, such as aqueous solutions of caustic soda, alkali metal carbonates and the like. The evolution of hydrogen halides is decidedly disadvantageous from the standpoint of equipment corrosion and general inconvenience. Treatment with strong bases, on the other hand, requires considerable caution to prevent excessive hydrolysis of the fat acid esters.

The reaction between certain halogen-containing organic compounds and aqueous solutions of salts of weak acids has heretofore resulted in substitution of the halogen group by a hydroxyl group. The chemical phenomenon of substitution is of no benefit in improving the

2

drying properties of long chain fatty acid compounds, and it normally requires a further step of dehydration in order to introduce unsaturated linkages in the long chain aliphatic radicals.

5 I have discovered that aqueous solutions of certain salts of weak acids are capable of effecting dehydrohalogenation of halogen-containing esters of the type previously mentioned. My results indicate that a certain amount of halogen substitution by hydroxy groups takes place concurrently with dehydrohalogenation, but have discovered the further remarkable fact that this phenomenon of substitution appears actually to increase the valuable drying properties of my 10 treated compounds.

I employ aqueous solutions of salts of acids having an ionization constant of  $2 \times 10^{-5}$  or less. The acids may be organic carboxylic acids or inorganic oxygen-containing acids; and examples of suitable salts are alkali metal acetates, borates, acid phosphates, propionates, maleates, valerates, acid pyrophosphates, malonates, bicarbonates, soaps of aliphatic long chain acids and the like. Salts other than alkali metal salts 15 20 may likewise be used, such as ammonium or amine salts, cupric, ferric, barium, calcium, magnesium, etc. Alkali metal salts are preferred, however.

The halogen-containing esters suitable in my process may be any long chain aliphatic acid esters, although my invention is particularly directed to esters of aliphatic polyhydric alcohols. Inasmuch as the specific method of halogenation appears to produce characteristic types of 25 30 halogen-containing compounds, I have determined by experimentation that any such compound may be employed so long as the contained halogen does not exist on adjacent carbon atoms in the aliphatic chain. I have discovered, however, that halogenated unsaturated glycerides produced by halogenating glyceride oils with certain positive halogen compounds, as disclosed in application Ser. No. 721,830, filed January 13, 35 40 45 1947, by Teeter and Cowan, now Patent No. 2,557,159, are especially adaptable to my process.

In general, according to that invention, the unsaturated higher fatty acid or its derivative is reacted under substantially anhydrous conditions with the alkyl hypohalite at a suitable temperature of about from 30° to 100° C. A solvent, such as carbon tetrachloride, benzene, chloroform, or petroleum ether may be employed, if desired. Reaction occurs rapidly and is complete in about from one to sixty minutes depend-

ing upon the temperature and the reactivity of the particular alkyl hypohalite employed.

The following example illustrates the halogenation method in accordance with said copending application. It will be understood, however, that halogenated esters prepared by other methods of halogenation are operative in the process so long as the halogen does not exist on adjacent carbon atoms in the aliphatic chain.

In a 500 ml. 3-necked flask equipped with thermometer, stirrer, and reflux condenser and kept in a constant-temperature bath at about 60° C., was placed 250 g. of alkali-refined soybean oil. By means of a dropping funnel having a long outlet tube extending through the reflux condenser to a point below the surface of the oil, 92 g. of tertiary butyl hypochlorite was added dropwise. An induction period of about

experiments. The reaction conditions are specified in the table, and it is to be noted that in all cases the unsaturation, particularly conjugated unsaturation is considerably increased. The 5 original oils, before halogenation and subsequent treatment by the process of my invention, contained negligible conjugated unsaturation. All dechlorinated oils possessed drying properties equal to or superior to refined linseed oil. Example 1 was a soybean oil control chlorinated with tertiary butyl hypochlorite by the process of the copending patent application previously referred to. Example 2 was a sample of methyl oleate chlorinated in the same manner. The 10 remainder of the examples were chlorinated soybean oil, also halogenated by the process previously referred to, all possessing halogen on non-adjacent carbon atoms of the acyl chains.

Table I

| Ex. No. | Time (Min.) | Temp. (°C.) | Press. (p. s. i.) | Reagent                                           | Chlorine Percent— |       | Gardner Color | Gardner Viscosity | Percent Hydroxyl | Total Conjugation Percent |
|---------|-------------|-------------|-------------------|---------------------------------------------------|-------------------|-------|---------------|-------------------|------------------|---------------------------|
|         |             |             |                   |                                                   | Before            | After |               |                   |                  |                           |
| 1.      |             |             |                   |                                                   | 8.96              | —     | 15-16         | J                 | —                | 20.9                      |
| 2.      | 60          | 195         |                   | 8% NaHCO <sub>3</sub>                             | 9.83              | 1.60  | —             | —                 | 1.3              | 28.7                      |
| 3.      | 60          | 195         |                   | 15% NaHCO <sub>3</sub>                            | 10.22             | 4.17  | —             | —                 | —                | 31.5                      |
| 4.      | 60          | 250         |                   | 15% NaHCO <sub>3</sub>                            | 10.22             | 1.43  | —             | —                 | —                | 32.9                      |
| 5.      | 30          | 250         |                   | 8% NaHCO <sub>3</sub>                             | 10.22             | 1.60  | —             | —                 | 1.2              | 25.0                      |
| 6.      | 30          | 250         |                   | 12% NaOOCCH <sub>3</sub>                          | 9.12              | 1.11  | 17-18         | D                 | 0.0              | 25.3                      |
| 7.      | 30          | 250         |                   | 32% Na <sub>2</sub> B <sub>7</sub> O <sub>7</sub> | 9.12              | 1.08  | 13            | E                 | 1.0              | 18.0                      |
| 8.      | 30          | 250         |                   | 18% Soap                                          | 9.12              | 0.99  | >18           | E                 | 0.8              | 31.5                      |
| 9.      | 100         | 233         | 440               | 8% NaHCO <sub>3</sub>                             | 1.04              | 0.67  | 17            | E                 | 1.2              | 28.9                      |
| 10.     | 85          | 237         | 440               | 12% NaOOCCH <sub>3</sub>                          | 9.06              | 2.34  | 14            | M                 | 2.0              | 28.8                      |
| 11.     | 87          | 240         | 440               | 16% Na <sub>2</sub> HPO <sub>4</sub>              | 9.06              | 2.72  | 14            | J                 | 1.6              | 22.9                      |
| 12.     | 84          | 244         | 460               | 17% Na <sub>2</sub> B <sub>7</sub> O <sub>7</sub> | 9.25              | 2.01  | 15            | T                 | 1.4              | 24.2                      |
| 13.     | 76          | 238         | 460               | 8% NaHCO <sub>3</sub>                             | 9.25              | 0.94  | 15            | R                 | 2.3              | 27.8                      |
| 14.     | 60          | 242         | 300               | Dry NaOOCCH <sub>3</sub>                          | 9.10              | 3.07  | >18           | W                 | 0.7              | 33.9                      |
| 15.     | 90          | 226         | 460               | 13.6% Na <sub>2</sub> HPO <sub>4</sub>            | 8.90              | 2.62  | 18            | J                 | 1.2              | —                         |

20 to 40 minutes, which terminated in a vigorous exothermic reaction, occurred upon initial addition of the hypochlorite. Following this period, the hypochlorite was added more rapidly. After all hypochlorite had been added, the reaction mixture was stirred at about 60° C. for about 60 minutes, in order to insure complete reaction. The reaction mixture was then stripped of volatile material by evacuating the flask at room temperature and passing an inert gas through the mixture for approximately two hours. The product contained 9.92 percent chlorine, and its viscosity and color, determined by Gardner standards, were H-I and 12-13, respectively. The product was further characterized by the presence of 14.6 percent diene, 5.1 percent triene, and 1.0 percent tetraene conjugation, determined spectrophotometrically. The total conjugation was 20.7 percent.

The following specific exemplary data illustrate my invention. It is to be understood that the specific conditions and reagents are not to be considered limiting. For example, the time of treatment may vary from 30 minutes up to several hours and the temperature of treatment may vary from 150° C. to 250° C. and higher. I prefer to employ autogenous pressure, but the process may be carried out at reflux temperatures or under excess pressure up to 500 pounds p. s. i. The concentration of the salt solution may vary over a wide range, for example, from 2½ percent up to the point of saturation. I prefer, however, to employ solutions of intermediate concentration as, for example 5 to 20 percent, when working with alkali metal salts. Less soluble salts I employ in concentrations approaching the point of saturation up to 10 to 15 percent.

Tabulated below are the results of a series of

40 The chlorinated soybean oil used in the examples tabulated above may be replaced by chlorinated cottonseed oil, chlorinated rapeseed oil, chlorinated oiticica oil, chlorinated safflower oil or chlorinated linseed oil. The chlorinated methyl oleate may be replaced by chlorinated ethyl lineoleate, chlorinated decyl oleate, or chlorinated oleic acid or linoleic acid.

45 I claim:

1. The method which comprises subjecting an ester of an aliphatic acid containing at least 8 carbon atoms in the acyl radical, said acid containing halogen substituted in the acyl radical and said substitution of halogen being upon non-adjacent carbon atoms, to the action of one of the group consisting of salts of organic carboxylic acids and salts of inorganic oxygen-containing acids, the acids of said salts possessing an ionization constant of less than  $2 \times 10^{-5}$ .

2. The method which comprises subjecting soybean oil, said oil containing halogen substituted in the acyl radical of the glyceride molecule and said substitution of halogen being upon non-adjacent carbon atoms, to the action of a 5-20 percent aqueous solution of one of the group consisting of salts of organic carboxylic acids and salts of inorganic oxygen-containing acids, the acids of said salts possessing an ionization constant of less than  $2 \times 10^{-5}$ .

3. Method of claim 2 in which the salt is sodium acid phosphate.

4. The method of increasing the conjugated olefinic unsaturation of a halogen containing 50 glyceride oil, said halogen being substituted in non-adjacent relationship upon the acyl radical, comprising subjecting said halogen containing glyceride oil to the action of an aqueous solution of a weakly basic salt of an acid possessing an ionization constant of less than  $2 \times 10^{-5}$ .

taken from the group consisting of organic carboxylic acids and inorganic oxygen-containing acids at a temperature in the range 150° C. to 250° C.

5. The method of increasing the conjugated olefinic unsaturation of a halogen containing soybean oil, said halogen being substituted in non-adjacent relationship upon the acyl radical of the glyceride molecule of the oil, comprising subjecting said oil to the dehalogenating action of an aqueous solution of a weakly basic salt of an acid possessing an ionization constant less than  $2 \times 10^{-5}$  taken from the group consisting of organic carboxylic acids and inorganic oxygen-containing acids.

6. Method of claim 5 in which the salt is sodium acetate.

7. Method of claim 5 in which the salt is sodium borate.

8. Method of claim 5 in which the salt is sodium acid phosphate.

9. The method which comprises increasing the conjugated olefinic unsaturation of chlorinated soybean oil, the chlorine being substituted in non-adjacent relationship upon the acyl radical of the oil glyceride, comprising subjecting said oil to the dechlorinating action of a 5 to 20 percent aqueous solution of a salt of the group consisting of  $\text{NaHCO}_3$ ,  $\text{NaOOCH}_3$ ,  $\text{Na}_2\text{B}_4\text{O}_7$ , and  $\text{Na}_2\text{HPO}_4$ .

10. The method of claim 9 in which the salt is sodium bicarbonate.

11. The method of claim 4 in which the halogen is chlorine.

HOWARD M. TEETER.

No references cited.